

## UNITED STATES PATENT OFFICE

ARTHUR W. BURWELL, OF NIAGARA FALLS, NEW YORK, ASSIGNOR TO ALOX CHEMICAL CORPORATION, OF NEW YORK, N. Y., A CORPORATION OF NEW YORK

## PENETRATING OIL COMPOSITION

No Drawing.

Application filed May 18, 1931. Serial No. 538,396.

This invention relates to oily compositions possessing pronounced penetrating and creeping properties, and to methods of preparing the same.

5 I have found that a composition having pronounced penetrating and creeping properties and adapted for loosening badly rusted nuts, bolts, studs and other parts of machinery, may be prepared by admixing a  
 10 light hydrocarbon oil such as the distillate known as kerosene with a small amount of a paraffin oil of relatively higher viscosity than kerosene and a small amount of a normally liquid mixture consisting essentially of alifatic saturated carboxylic acids of mineral origin substantially identical with the acidic mixture obtainable by treating with aqueous alkali solution a reaction mass containing both saponifiable and unsaponifiable components produced by the controlled liquid-phase partial oxidation of a petroleum distillate known as "45° distillate", or "fuel oil distillate", or gasolines, or naphthenes, or other hydrocarbon mixtures consisting  
 15 essentially of hydrocarbons whose molecular weights are above those corresponding to 7 or 8 carbon atoms in the molecule, at elevated temperature and pressure in the presence of an inciter of oxidation, separating  
 20 the resulting soaps in solution from the unsaponified components, precipitating the soap acids from the solution, and subjecting the precipitated soap acids to distillation treatment at a temperature of from about  
 25 280° C. to about 300° C. whereby to obtain an acidic distillate fraction consisting essentially of saturated alifatic carboxylic acids having an average molecular weight of from 160 to 165, and a range of carbon atoms in  
 30 the molecule of from 4 to 12.

I have found that the addition of the aforesaid acidic mixture to a low-viscosity petroleum-distillate such as kerosene or the distillate known as "Varnolene" either with  
 35 or without addition thereto of a minor proportion of a higher viscosity oil having lubricating properties, such for instance as paraffin oil, pronouncedly enhances the penetrating and creeping properties of the said  
 40 distillate, or of the said mixture, the result-

ing composition creeping extremely rapidly on the surface of any metal or of any composition containing metals even in the oxidized form (e. g., on glass).

An illustrative example of compositions embodying the present invention is the following:

|                                                               | Per cent |
|---------------------------------------------------------------|----------|
| Kerosene, water-white                                         | 72       |
| The aforesaid acidic mixture                                  | 1-3 60   |
| Paraffine oil, having a viscosity of about 150 at 100 Saybolt | 27-25    |

The composition is simply prepared, it being necessary to combine the ingredients which are freely soluble in each other.

Considerable variation in the proportions of the ingredients, and in the ingredients themselves, may be made without departing from the spirit of the invention. Thus, in the above example, the proportion of the paraffine oil ingredient may be diminished, with corresponding increase in the proportion of the kerosene. The function of the paraffin oil ingredient is to confer "oiliness" and lubricating properties upon the mixture; therefore, in cases where lubrication is not desired the said ingredient may be omitted altogether. For the kerosene there may with equal success be substituted a corresponding amount of "Varnolene" or other light, low-viscosity, petroleum distillate such as the furnace oil used in domestic oil-heating plants. For the specific paraffin oil above identified there may be substituted another lubricating oil having a relatively high viscosity. Also, for the aforesaid acidic mixture there may, with substantially as good results, be substituted in part other acidic mixtures obtained by the controlled, liquid-phase, partial oxidation of other petroleum hydrocarbon mixtures with subsequent separation of the acidic products from non-acidic oxidation products and unoxidized hydrocarbons, which acidic mixtures may or may not have been subjected to the aforesaid distillation treatment and contain or consist of a plurality of acids having varying molecular weights.

I claim:

1. A penetrating oil composition comprising in major proportion a light low-viscosity petroleum distillate and a relatively small but effective amount of a normally liquid acidic mixture insoluble in water but freely soluble in said distillate and consisting essentially of alifatic saturated carboxylic acids, of mineral origin, having a range of carbon atoms in the molecule of from 4 to 12 and an average molecular weight of from 160 to 165.
2. A penetrating oil composition comprising in major proportion a light low-viscosity petroleum distillate, in minor proportion a lubricating oil miscible with the said distillate, and a relatively small but effective amount of a normally liquid acidic mixture insoluble in water but freely soluble in said distillate and consisting essentially of alifatic saturated carboxylic acids, of mineral origin, having a range of carbon atoms in the molecule of from 4 to 12 and an average molecular weight of from 160 to 165.
3. A penetrating oil composition as defined in claim 1, in which the petroleum distillate is kerosene.
4. A penetrating oil composition as defined in claim 2, in which the petroleum distillate is kerosene, the lubricating oil is a 25° paraffin oil having a viscosity of about 150 at 100 Saybolt, and in which the ingredients are present in about the proportion of 72% kerosene, 1 to 3% of the aforesaid acidic mixture, and 27 to 25% paraffin oil.
5. A penetrating oil composition comprising in major proportion a light low-viscosity petroleum distillate and a relatively small but effective amount of a normally liquid acidic mixture insoluble in water but freely soluble in said distillate and consisting essentially of alifatic saturated carboxylic acids, of mineral origin.
6. A penetrating oil composition as defined in claim 5, in which the petroleum distillate is kerosene.

In testimony whereof, I affix my signature.

ARTHUR W. BURWELL.